

# UNITED STATES PATENT OFFICE.

FIN SPARRE, OF WILMINGTON, DELAWARE, ASSIGNOR TO THE E. I. DU PONT DE NEMOURS POWDER COMPANY, OF WILMINGTON, DELAWARE, A CORPORATION OF NEW JERSEY.

## EXPLOSIVE.

No. 852,143.

Specification of Letters Patent.

Patented April 30, 1907.

Application filed September 11, 1906. Serial No. 334,083.

*To all whom it may concern:*

Be it known that I, FIN SPARRE, a subject of the King of Norway, residing at Wilmington, county of Newcastle, and State of Delaware, have invented a new and useful Improvement in Explosives, of which the following is a full, clear, and exact description.

I have discovered that tetranitrodiglycerin,  $C_6H_{10}O(ONO_2)_4$ , possesses several excellent properties making it very well suited as an ingredient of smokeless powder. It is insensitive to blows and friction, making its own manufacture, and the manufacture of explosives containing it, comparatively safe. It is an excellent solvent for nitrocellulose and makes a splendid colloid without application of a volatile solvent. It is non-freezing at temperatures met with in practice, so that explosives containing tetranitrodiglycerin keep their strength in the winter, and it does not exude from the powder grains.

My invention consists of an explosive composition or smokeless powder containing, in addition to tetranitrodiglycerin, nitrocellulose and preferably also nitroglycerin and nitrotoluol.

Dinitroglycerin has been suggested as an ingredient for smokeless powder with a view of making a non-freezing nitroglycerin smokeless powder, but dinitroglycerin is not stable enough, as it gives off nitrous fumes above 50 degrees centigrade. Dinitrochlorhydrin has also been suggested but it cannot be practically used, because hydrochloric acid, causing corrosion of the gun, is evolved by its combustion. None of these objections is applicable to tetranitrodiglycerin.

Tetranitrodiglycerin is formed by the nitration of diglycerin, the process being substantially the same as the nitration of glycerin to form the ordinary trinitroglycerin.

In my invention, tetranitrodiglycerin may be used with or without mixture with ordinary nitroglycerin. The manufacture of smokeless powder containing tetranitrodiglycerin does not differ from known processes. A preferred way is to mix the wet nitrocel-

lulose with the tetranitrodiglycerin and the other ingredients, if any, in the presence of 50 water and steam, after which they are dried and colloided on hot rolls.

The following are preferred compositions embodying my invention.

I. Nitrocellulose 40 to 65%, preferably 55 50%, tetranitrodiglycerin 35 to 60%, preferably 50%.

II. Nitrocellulose 40 to 65%, preferably 50%, nitroglycerin less than 50%, preferably 30%, tetranitrodiglycerin more than 5%, 60 preferably 20%.

III. Nitrocellulose 40 to 65%, preferably 48%, trinitrotoluol less than 25%, preferably 12%, nitroglycerin less than 40%, preferably 25%, tetranitrodiglycerin more than 5%, 65 preferably 15%.

IV. Nitrocellulose 40% to 65%, preferably 55%, vaseline less than 10%, preferably 5%, trinitrotoluol more than 15%, preferably 25%, nitroglycerin less than 25%, 70 preferably 10%, tetranitrodiglycerin 2 to 20%, preferably 5%.

V. Nitrocellulose 40 to 70%, preferably 60%, trinitrotoluol 10 to 50%, preferably 30%, tetranitrodiglycerin 5 to 30%, 75 preferably 10%.

In case vaseline is used, it may be first dissolved in the tetranitrodiglycerin before mixing with the other ingredients as before described.

In an application of even date herewith, Serial No. 334,082, I have set forth the use tetranitrodiglycerin as an ingredient of blasting explosives, but my present invention is confined to its use as an ingredient 85 of smokeless powder.

Having now fully described my invention, what I claim and desire to protect by Letters Patent is:

1. An explosive containing nitrocellulose 90 and tetranitrodiglycerin substantially as described.

2. An explosive containing nitrocellulose, nitroglycerin and tetranitrodiglycerin substantially as described.

3. An explosive containing nitrocellulose,

95

nitroglycerin, trinitrotoluol and tetranitrodiglycerin substantially as described.

4. An explosive containing nitrocellulose, trinitrotoluol and tetranitrodiglycerin substantially as described.

5. An explosive containing nitrocellulose, nitroglycerin, trinitrotoluol, tetranitrodiglycerin and vaseline substantially as described.

6. An explosive containing nitrocellulose

and less than 60% of tetranitrodiglycerin to substantially as described.

In testimony of which invention, I have hereunto set my hand, at Wilmington, on this 7th day of Sept., 1906.

FIN SPARRE.

Witnesses:

FRANK H. MASON,  
S. M. MUNDA.